

## UNITED STATES PATENT OFFICE.

JAMES EDWIN GEE AND FREDERICK SAMUEL GEE, OF LONDON, ENGLAND.

## HEAT TREATMENT OF PERMANENT MAGNETS.

No Drawing. Application filed March 21, 1925, Serial No. 17,440, and in Great Britain March 25, 1924.

The present invention relates to a method of making permanent magnets by casting from metal melted in a crucible or by a process which does not add materially to the carbon contents of the metal, and heat treatment before magnetizing.

According to this invention the heat treatment consists in first softening and then hardening the castings.

10 In applying the invention to the manufacture of letters or characters used for display devices, the letters or characters are preferably cast with feet which are positioned so that when they are magnetized the feet 15 form the magnetic poles. We prefer to provide each character with more than one pair of feet as by this means a stronger magnetic attraction is obtained as explained in our prior patent specification No. 1,464,740 (Re- 20 issue No. 15,847). The characters are then softened, hardened and magnetized.

As an example, the following heating treatment is adopted when steels containing cobalt are used for the magnets. A preferred 25 steel is one containing 9 to 15 per cent of cobalt and 9 to 15 per cent of chromium, but any steel usually known as cobalt steel may be employed. To soften the castings they are raised to a temperature of approximately 30 650 degrees C., and the heat maintained for about half-an-hour when they are allowed to cool.

The hardening treatment consists of three successive heatings and coolings before magnetizing. The first heating is to approximately 35 1,200 degrees C., after which the castings are cooled off and allowed to remain for about 18 hours. In the second treatment the castings are re-heated to approximately 750 40 degrees C., and they are again allowed to cool. The castings are then finally heated to approximately 1,000 degrees C., for about

ten minutes and again allowed to cool. It is preferable to let the castings remain for about twelve hours after the final heating 45 process before magnetizing. After magnetizing they will be found to be permanent magnets.

Although the invention has been described applied to the manufacture of letters or characters for display devices, it will be understood that it can be employed for making permanent magnets for any other purpose.

What we claim is:—

1. A method of making permanent magnets by casting and heat treating the castings only before magnetizing, in which the castings are softened by heating and then hardened by first heating to approximately 1,200° C., then cooling and leaving for about 60 18 hours, reheating to approximately 750° C., and allowing to cool and finally heating to approximately 1,000° C. for ten minutes, allowing to cool, and leaving for about 12 65 hours before magnetizing.

2. A method of making permanent magnets by casting cobalt steel and heat treating the castings only before magnetizing, in which the castings are softened by heating to approximately 650° C. and maintaining 70 the temperature for half-an-hour, then allowing the castings to cool, and then hardened by first heating to approximately 1,200° C., then cooling and leaving for about 18 hours, reheating to approximately 750° C. 75 and allowing to cool and finally heating to approximately 1,000° C. for ten minutes, allowing to cool, and leaving for about 12 hours before magnetizing.

In testimony whereof we have signed our 80 names to this specification.

JAMES EDWIN GEE.  
FREDERICK SAMUEL GEE.